

J. K. TOLES.  
BELT RAIL.  
APPLICATION FILED JULY 8, 1919.

1,333,141.

Patented Mar. 9, 1920.



Fig. 1.



Fig. 2.



Fig. 3.

WITNESS  
G. S. Goores.

INVENTOR  
J. K. Toles

BY *White & Pratt*

ATTORNEYS

# UNITED STATES PATENT OFFICE

JUSTIN KAY TOLES, OF SAN FRANCISCO, CALIFORNIA.

## BELT-RAIL.

1,333,141.

Specification of Letters Patent. Patented Mar. 9, 1920.

Application filed July 8, 1919. Serial No. 309,438.

To all whom it may concern:

Be it known that I, JUSTIN KAY TOLES, a citizen of the United States, and a resident of the city and county of San Francisco and State of California, have invented a new and useful Belt-Rail, of which the following is a specification.

My invention relates to belt rails for refrigerator cars.

10 An object of the invention is to provide a belt rail with which the insulating layers may be secured on the walls of a refrigerating car, and which greatly retards the conduction of heat therethrough, thus making 15 the heat insulating material continuous, instead of arranging it in strips separated by non-insulating material as is the case when wooden belt rails are used.

20 The invention possesses other features of advantage, some of which, with the foregoing, will be set forth in the following description of the preferred form of my invention which is illustrated in the drawings accompanying and forming part of the 25 specification. It is to be understood that I do not limit myself to the showing made by the said drawings and description, as I may adopt variations of the preferred form within the scope of my invention as set 30 forth in the claims.

Referring to the drawings:

Figure 1 is a perspective view of a piece of belt rail made in accordance with my invention.

35 Fig. 2 is a vertical section taken transversely through a portion of a refrigerator car wall, showing how the belt rail of my invention is applied.

40 Fig. 3 is a transverse section through a modified form of belt rail.

The belt rail of my invention comprises a built up shape as shown in Fig. 1 formed by adhesively securing together layers or sheets of fiberized and felted material, preferably rice straw. Alternate layers 2 are formed of relatively densely packed or felted fibers giving a hard sheet, and the intervening layers 3 are formed of relatively loosely packed fibers giving a soft sheet.

45 In the making of the hard sheets, the straw is first fiberized in any suitable manner, as by cooking in an alkaline solution, and then macerated and washed. A suitable amount of the floating fiber is then ac-

cumulated in a layer of relatively uniform 55 thickness on a foraminous surface, the water being allowed to drain away. The material is then suitably worked to bring the smaller and finer fibers to the surface of the layer, to form a skin of finer texture than the interior of the layer. The skins being of finer texture and less porous than the interior of the layer retard or break up convection currents tending to pass through the material. The layers are finally pressed to condense 65 the fibers and form a relatively stiff hard sheet which is then cut up into strips of the desired size. The making of the soft sheets is similar but they are not pressed, the fibers being merely loosely matted or felted together and worked to create the surface skin of fine fibers.

When these sheets are secured together in alternate layers, the laminated structure provides a plurality of surface skins which 75 break up and retard the flow of heat through the structure, providing much greater heat insulating value, than would be found in a homogeneous structure of the same size. The loosely felted fibers permit convection 80 currents, diverted by the skins and dense layers to pass outwardly to the edges of the rail. The desired number of alternate layers of hard and soft material, as for instance five, as shown in Fig. 1 are adhesively 85 secured together to form the main body of the rail, hard layers being preferably disposed on the outside. A similar composite structure of adhesively united alternate layers of hard and soft sheets, 5 and 6 respectively, but narrower than the main body 90 is cemented to the main body, so that rabbeted edges are formed longitudinally of the belt rail, in which the edges 7 of the insulating layers 8 are adapted to lie. The 95 edges 7 are thus condensed and securely held between the ship lap siding 9 and the belt rail, which is secured in position in any suitable way as by nails. The thickness of the belt rail is such as to bring its 100 outer surface flush against the tongue and groove sheathing 12.

The belt rail thus comprises a laminated structure formed of alternate layers of hard and soft fibrous materials, each formed 105 with a surface skin of finer texture, and having adjacent edges of the structure rabbeted. To accord with this definition,

the contiguous hard layers 2 and 5 in Fig. 1 may be considered as one, or if desired, the contiguous layer 5 may be omitted, the succeeding soft layer 6 lying contiguous to the outer hard layer 2.

In Fig. 3 I have shown a modified form of belt rail in which strips 13 of densely felted material are cemented to the edges of the belt rail, thus completely inclosing the edges of the strips, and retarding the movement of convection currents through the loosely felted layers.

I claim:

1. A belt rail comprising a laminated structure formed of layers of fiberized and felted material.
2. A belt rail comprising a laminated structure formed of layers of fiberized and felted cereal straw.
3. A belt rail comprising a laminated structure formed of layers of fiberized and felted material adhesively united, each layer having a skin which retards heat convection in greater degree than the interior of the layer.
4. A belt rail comprising a laminated structure formed of layers of fiberized and felted material adhesively united, each layer having a skin which retards heat convection in greater degree than the interior of the layer, and said layers being narrower on

one side of the structure whereby rabbets are formed along adjacent edges thereof.

5. A belt rail comprising a laminated structure formed of layers of fiberized and felted material, and having adjacent longitudinal edges rabbeted.

6. A belt rail comprising a laminated structure formed of layers of densely and loosely felted fibrous material.

7. A belt rail comprising a laminated structure formed of densely and loosely felted fibrous material in alternate layers.

8. A belt rail comprising a laminated structure formed of densely and loosely felted fibrous material in alternate layers and having adjacent longitudinal edges rabbeted.

9. A belt rail comprising a laminated structure formed of layers of densely and loosely felted fibrous material formed with a surface skin of finer fibers on each layer.

10. A belt rail comprising a laminated structure formed of adhesively united layers of fiberized and felted material, and a layer of similar material adhesively united to and contiguous with the edges of said layers.

In testimony whereof I have hereunto set my hand at San Francisco, California, this 27th day of June, 1919.

JUSTIN KAY TOLES.